

United States Patent [19]  
Küffner et al.

[11] 3,849,140  
[45] Nov. 19, 1974

- [54] DIFFUSION-RESISTANT DISPERSIBLE  
YELLOW COUPLERS FOR THE  
PRODUCTION OF PHOTOGRAPHIC  
COLOR IMAGES
- [75] Inventors: **Karl Küffner**, Unterhaching near  
Munich; **Hans Glockner**, Pullach  
near Munich, both of Germany
- [73] Assignee: **Agfa-Gevaert Aktiengesellschaft**,  
Leverkusen, Germany
- [22] Filed: **Mar. 22, 1972**
- [21] Appl. No.: **236,972**

- [30] Foreign Application Priority Data  
Mar. 25, 1971 Germany ..... 2114577
- [52] U.S. Cl. ..... 96/100, 96/74, 260/262 R  
[51] Int. Cl. ..... G03c 1/40  
[58] Field of Search ..... 96/100
- [56] References Cited  
UNITED STATES PATENTS  
3,409,439 11/1968 Yoshida et al. ..... 96/100

3,725,072 4/1973 Yoshida et al. ..... 96/100

Primary Examiner—J. Travis Brown  
Attorney, Agent, or Firm—Connoly and Hutz

[57]

ABSTRACT

A multiple-layer color photographic material containing silver halide as the photo-sensitive substance containing in the blue-sensitive component layer a diffusion resistant dispersible color coupler for the formation of the yellow partial image of the following formula



wherein the substituents

R<sub>1</sub>, X, R<sub>2</sub> and n have the same definition as  
described hereinafter, which developed dye have  
favorable spectral properties.

3 Claims, No Drawings

DIFFUSION-RESISTANT DISPERSIBLE YELLOW  
COUPLERS FOR THE PRODUCTION OF  
PHOTOGRAPHIC COLOR IMAGES

This invention relates to color couplers which react with suitable developer substances of the p-phenylene diamine type to form yellow dyes according to the principle of chromogenic development. These color couplers are preferably used in the blue-sensitive component layer of multiple-layer color photographic materials containing silver halide as the photosensitive substance.

As already known, derivatives of benzylacetanilide are mainly used as color couplers for the aforementioned purpose. The properties of the couplers, and of the dyes formed from them, can be influenced within wide limits by suitable substituents at various positions in the molecule. Thus, the introduction of relatively long hydrocarbon radicals makes the compounds resistant to diffusion, so that they can be embedded in the blue-sensitive component layer of the multiple-layer colour material. The effect of introducing a sulfo group or carboxyl group into the molecule is that the colour couplers can be added to the silver halide emulsion in the form of water-soluble alkali metal salts. The effect of substitution of the reactive methylene group with halogen, or any other radical which can be split off during color coupling, is that only two molecules of silver halide, rather than four, are required for dye formation (the color couplers are then so-called 2-equivalent couplers). Finally, other substituents may be necessary in order to improve the photographic properties of the coupler and of the dye formed therefrom.

The present invention relates to diffusion-resistant water-insoluble yellow couplers which are used in dispersed form. The requirements which must be satisfied by couplers such as these are extremely varied, the following being mentioned by way of example: high solubility in certain organic solvents and a relatively low melting point with a consequent high dispersibility in water or gelatin solution; high resistance to diffusion, stability of the coupler against climatic influences during storage of the finished color materials; limited influence upon the photographic properties of the silver halide; high reactivity during color development; favourable spectral properties of the developed dye; and resistance of the image dye to light and climatic influences. Last but not least, the coupler should be easy to prepare, thus minimising production costs.

It now has been found that benzylacetanilides having the general formula (I) are eminently suitable for the production of yellow coupler images:



wherein:

R<sub>1</sub> represents a diffusion-inhibiting radical in the form of a linear or branched hydrocarbon chain having at least 10 carbon atoms;

X represents hydrogen or a radical which can be split off during colour coupling, mostly chlorine;

R<sub>2</sub> represents halogen, cyano, R<sub>3</sub>, OR<sub>3</sub>, CF<sub>3</sub>, COOR<sub>3</sub>, CONH<sub>2</sub>, CONHR<sub>3</sub>, CON(R<sub>3</sub>)<sub>2</sub>, SO<sub>2</sub>R<sub>3</sub>, SO<sub>2</sub>NH<sub>2</sub>, SO<sub>2</sub>NHR<sub>3</sub>, SO<sub>2</sub>N(R<sub>3</sub>)<sub>2</sub>, or SO<sub>2</sub>F; and if two or more radicals R<sub>2</sub> are present, they can be the same or different;

R<sub>3</sub> represents alkyl having 1 to 4 carbon atoms or aryl, and if two groups R<sub>3</sub> occur in the same radical, they can be the same or different; and

n represents 1, 2 or 3.

10 The particular characteristic of these couplers is the presence of a diffusion-inhibiting radical in the form of a long-chain alkoxy group in the ortho-position of the benzoyl radical. Couplers in which one group R<sub>2</sub> represents a chlorine atom in the ortho-position, are particularly suitable. Accordingly, couplers of this kind have the formula (II):



20 in which R<sub>1</sub>, R<sub>2</sub>, X and n have the meanings given above. The effectiveness of couplers used according to the invention results in conjunction with the aforementioned substituents in the anilide portion. This is particularly true as regards 2-equivalent couplers having chlorine as the separable radical.

25 Large numbers of dispersible couplers in which the diffusion-inhibiting radical is linked otherwise than through an O-atom to the molecule, or is attached anywhere to the molecule, have previously been described. Compared with the substances used according to the invention, all these couplers show a greater tendency towards crystallisation and, for this reason, they can often only be used in conjunction with oil formers. Although this disadvantage can be obviated by introducing a water-solubilising group (for example a sulfo group) into the molecule, this measure has an adverse effect upon the spectral properties of the image dyes developed therefrom, since it displaces absorption towards longer wavelengths, and at the same time the definition of the color image is impaired.

30 35 40 45 50 The favourable effect of ortho-methoxy substitution in the benzoyl radical upon the spectral properties of the image dyes is also known. This is described in U.S. Pat. No. 2,728,658 to McCrossen et al. This has not, however, acquired any real practical significance because numerous preparative difficulties are involved in producing the o-methoxybenzoyl-acetic esters.

55 60 65 Comparison of the couplers used according to the invention, with couplers in which an alkoxy group is situated in the para-position of the benzoyl radical, is of particular significance. This para-alkoxy substitution leads to extremely active couplers which have, however, disadvantages in comparison with the couplers used according to the invention, including longer-wave absorption of the developed dyes and lower solubility, for example in ethyl acetate. The melting points of couplers having a long-chain alkoxy substituent in the para-position are from 10° to 40°C higher than the melting points of the corresponding couplers with the long-chain alkoxy substituents in the ortho-position. Because of this property, these para-alkoxy couplers are more difficult to disperse, in addition to which they crystallise more readily from dispersions. In addition 2-equivalent couplers produced from couplers such as

these generally show a tendency towards heavy yellow fogging. When a water-solubilising group is introduced into para-alkoxybenzoyl couplers, an unfavourable displacement of the absorption maximum of the dyes towards longer wavelengths is obtained in this instance also.

The following are examples of the couplers used according to the invention:



10



20



30



35

40



45

50



55



65



- 5
16. 
24. 
- 10
17. 
25. 
- 15
18. 
- 20
26. 
- 25
19. 
- 30
27. 
- 35
20. 
- 40
28. 
- 45
21. 
- 50
29. 
- 55
22. 
- 60
30. 
- 65
23. 
31. 

7



8



3,849,140

9



10



10



20



30



40



45



55



60



65





The process for producing the new couplers is known in principle and comprises reacting suitably substituted aniline derivatives with long-chain o-alkoxybenzoyl acetic esters. It is worth noting that these esters can be produced relatively easily compared with o-methoxy-benzoyl acetic esters which are much more difficult to obtain. The coupler obtained can be subsequently converted into a 2-equivalent coupler, also by known methods.

The new couplers can readily be introduced into a silver halide emulsion. The dispersions are prepared by known methods. The most common method is to prepare a solution in water or gelatin solution with the assistance of a suitable wetting agent, and then to evaporate off the solvent. If necessary, a so-called oil former can be added in order to prevent crystallisation. There is, however, generally no need to do this with the couplers according to the invention, because of their particularly high dispersibility. The disadvantages of using oil formers are known.

The new yellow couplers react really well with the oxidation products of all conventional developers of the p-phenylene diamine type, for example N,N-diethyl-p-phenylene diamine (CD 1), N,N-diethyl-3-methyl-p-phenylene diamine (CD 2), 4-amino-3-methyl-N-ethyl-N-methane sulphonamidoethyl aniline (CD 3), N-ethyl-N-β-hydroxyethyl-3-methyl-p-phenylene diamine (CD 4), and N-butyl-N-δ-sulphobutyl-p-phenylene diamine (T 60).

The developed dyes absorb at relatively short wavelengths. Secondary absorption in the green region of the spectrum is minimal.

The properties of the 2-equivalent couplers used according to the invention, especially with chlorine as the

separable radical, are particularly remarkable. During color development, these couplers cause little or no color fogging, a property which distinguishes them with advantage from most of the 2-equivalent couplers which have been described. The components according to the invention can be used both in the negative-positive process and also in the reversal process. Both film and paper can be used as layer substrate for the layers.

Representative couplers according to the invention can be prepared as follows:

1. Coupler 13

a. Methyl 2-tetradecyloxybenzoate

23 g of sodium metal were dissolved in 500 ml of ethylene glycol monomethylether, followed by the addition

20

35 tion of a solution of 125 g of methyl salicylate in 400 ml of ethylene glycol monomethylether. The resulting mixture was then brought to boiling while stirring, followed by the dropwise addition of 277 g of tetradecyl bromide over a period of 3 hours. The mixture was then boiled for another hour, after which it was left to cool.

40 After stirring into 3 litres of water, the oil which precipitated was taken up in ether, and the ethereal solution was dried and evaporated, leaving behind a brown oil which was distilled in vacuo.

45 B.p. <sub>0.15</sub> 198° – 199°C. Yield: 213 g (61% of the theoretical)

b. 2-tetradecyloxybenzoic acid

50 213 g of methyl 2-tetradecyloxybenzoate were dissolved in 500 ml of ethanol, followed by the addition of a solution of 91 g of potassium hydroxide in 90 ml of water. After boiling under reflux for 1 hour, the mixture was stirred into 3 litres of water and acidified with 10% by weight hydrochloric acid.

55 The acid which was precipitated was filtered under suction and washed with water. Recrystallization from methanol gave 163 g (80% of the theoretical) of pure acid. M.P. 51°C.

c. 2-tetradecyloxybenzoyl chloride

60 162 g of acid were fused and 100 ml of thionyl chloride were added in portions to the resulting melt. The reaction mixture was heated until the internal temperature had reached 100°C.

65 Excess thionyl chloride was then distilled off in vacuo. The acid chloride solidified.

Yield: 166 g (97% of the theoretical) M.p. 34° – 35°C.

d.  $\alpha$ -(2-tetradecyloxybenzoyl) acetoacetic ethyl ester

173 g of the acid chloride dissolved in 50 ml of benzene were added with stirring to 150 g of sodium aceto-

acetic ethyl ester suspended in 50 ml of benzene. After boiling for 3 hours, the benzene was evaporated off, and the residue was poured into 2 litres of ice water and acidified with 10% by weight hydrochloric acid. The oil which was precipitated was extracted with ether, and the ethereal solution was washed, dried and evaporated.

Yield: 198 g (90% of the theoretical) M.p. 44° - 45°C.

e. Methyl 2-tetradecyloxybenzoyl-acetate

251 g of  $\alpha$ -(2-tetradecyloxybenzoyl) acetoacetic ethyl ester, 135 g of 30% by weight sodium methoxide solution and 120 ml of methanol were boiled for 2.5 hours. After standing overnight, the mixture was poured into 2 litres of water, acidified and extracted with ether.

Evaporation of the ethereal solution left 193 g of ester, (96% of the theoretical) M.p. 40° - 41°C.

f. 2-tetradecyloxybenzoyl-4'-methyl-acetanilide

10.7 g of 4-aminotoluene (p-toluidine) and 39.0 g of methyl 2-tetradecyloxybenzoyl-acetate were boiled for 6 hours in 100 ml of xylene, the alcohol which was eliminated ( $\text{CH}_3\text{OH}$ ) being distilled off through a short column.

The residue was then dissolved hot in 500 ml of methanol, filtered and left to crystallize.

Yield: 37.9 g M.p. 92° - 93°C

2. Coupler 14

2-tetradecyloxybenzoyl-4'-methyl-chloroacetanilide

5.2 g of sulfonyl chloride dissolved in 20 ml of chloroform were added dropwise over a period of 30 minutes, while stirring and cooling with ice water (2°C), to 18 g of coupler 13 dissolved in 200 ml of chloroform. The mixture was then stirred for 1 hour in ice water, and then for a further hour at room temperature.

The chloroform was evaporated off in vacuo and the residue was recrystallized from 300 ml of methanol.

Yield: 14 g M.p. 95° - 97°C.

Chlorine determination:

found 6.9% Cl

calculated 7.1% Cl

3. Coupler 17

2-tetradecyloxybenzoyl-2'-methoxy-acetanilide

This coupler was prepared in accordance with Specification 1f, except that 13.5 g of o-anisidine were used instead of the 4-amino toluene.

Yield: 22.4 g M.p. 58° - 60°C.

4. Coupler 18

2-tetradecyloxybenzoyl-2'-methoxy-chloroacetanilide

This coupler was prepared in accordance with Specification 2, except that, instead of coupler 13, 24.2 g of coupler 17 were reacted with 6.75 g of sulfonyl chloride.

Yield: 23.4 g M.p. 43° - 45°C.

5. Coupler 19

2-tetradecyloxybenzoyl-2'-methoxy-fluoroacetanilide

A three-necked flask equipped with stirring mechanism, thermometer and gas-inlet pipe, was filled with 300 ml of methanol. The methanol was cooled to -40°C with acetone/dry ice. Perchloryl fluoride was then introduced until the methanol contained 5.5 g of perchloryl fluoride.

A solution of 24 g of coupler 17 in 125 ml of methanol 9.1 g of 30% by weight sodium methoxide solution were run into the aforementioned perchloryl fluoride solution over a period of 30 minutes at -30°C. The temperature was kept at -20°C.

After 15 minutes, 300 g of ice water were added and the coupler that was precipitated was filtered off under suction, washed with water, and recrystallized twice

from methanol.

Yield: 18.4 g M.p. 56° - 57°C

Fluorine determination:

Calculated 3.8% F

found: 4.0% F

6. Coupler 20

2-tetradecyloxybenzoyl- $\alpha$ -4'-nitrophenoxy-2''-methoxy-acetanilide

10.3 g of coupler 18, 3.3 g of sodium 4-nitrophenoxy and 350 ml of acetonitrile were boiled under reflux for 7 hours. After the solvent had been distilled off in vacuo the residue was dissolved in a little methanol and the resulting solution was poured into 300 ml of ice water. The oil that was precipitated solidified when triturated with a little methanol.

6 g of coupler were obtained after two recrystallizations from methanol. M.p. 59° - 64°C.

7. Coupler 41

2-tetradecyloxybenzoyl-2'-chloro-5'-N-methyl sulfamyl-acetanilide

This coupler was prepared in accordance with Specification 1f, except that 22 g of 2-chloro-5-N-methylsulfamyl-aniline were used instead of the 4-amino toluene.

Yield: 40 g M.p. 90° - 92°C.

25 8. Coupler 42

2-tetradecyloxybenzoyl-2'-chloro-5'-N-methylsulfamylchloroacetanilide

This coupler was prepared in accordance with Specification 2, except that, instead of coupler 13, 29 g of coupler 41 were reacted with 6.75 g of sulfonyl chloride.

Yield: 23.4 g M.p. 84° - 86°C.

Chlorine determination:

11.56% Cl calculated

35 11.3% Cl found

9. Coupler 48

2-tetradecyloxybenzoyl-4'-methylsulfonyl-acetanilide

This coupler was prepared in accordance with Specification 1f, except that 17.1 g of 4-methylsulfonyl-aniline were used instead of 4-amino-toluene.

Yield: 35 g M.p. 79° - 80°C.

19. Coupler 49

2-tetradecyloxybenzoyl-4'-methylsulfonyl-chloroacetanilide

45 This coupler was prepared in accordance with Specification 2, except that, instead of coupler 13, 26.5 g of coupler 48 were reacted with 6.75 g of sulfonyl chloride.

Yield: 18.2 g M.p. 94° - 96°C.

50 Chlorine determination:

Calculated 6.41% Cl

found 6.2% Cl

The following Examples illustrate the invention.

EXAMPLE 1

a. Preparation of a dispersion of coupler 17.

1.93 g of coupler were dissolved in 10 ml of ethyl acetate and the resulting solution was stirred intensively into 150 ml of 7.5% by weight gelatin solution containing 0.25 g of sodium dodecylbenzene sulfonate. Dispersion time was 2 minutes, a Kotthoff mixing siren being used for dispersion. The ethyl acetate was evaporated off on a water bath. This dispersion could be stored for several days without change, either in liquid form or in solid form.

65 b. Photographic application.

The above dispersion was added to 50 g of a negative emulsion. The silver content, expressed as  $\text{AgNO}_3$ , was 4.08 g. Following addition of the usual casting additives, the emulsion was cast onto a layer substrate and

dried. Thereafter, samples were exposed under a step wedge (blue filter) both fresh and after cold storage (for 7 days at  $-20^{\circ}\text{C}$ ). The samples were subjected to a negative development process (developer substance: diethyl-p-phenylene diamine). The following measurements were obtained:

|                    | relative sensitivity | density | fogging |
|--------------------|----------------------|---------|---------|
| fresh              | 100                  | 1.81    | 0.12    |
| after cold storage | 100                  | 1.79    | 0.12    |

The following Table shows the absorption maxima of the dyes obtained from coupler 17 with different developer substances, mentioned in the description.

|      | nm  |
|------|-----|
| CD 1 | 420 |
| CD 2 | 427 |
| CD 3 | 425 |
| T 60 | 422 |

c. Comparison test with the coupler:



In this coupler, the two alkyl radicals have been interchanged compared to coupler 17 used according to the invention. The dispersion was prepared and the photographic emulsion was applied as in (a) and (b). The following measurements were obtained:

|                    | relative sensitivity | density | fogging |
|--------------------|----------------------|---------|---------|
| fresh              | 100                  | 1.40    | 0.12    |
| after cold storage | 60                   | 0.98    | 0.10    |

In contrast to (b), a marked reduction in sensitivity and density is observed after cold storage in this instance. This is attributable to crystallization of the coupler.

EXAMPLE 2

a. A dispersion was prepared from 2.06 g of coupler 18 in the manner described in Example 1a.

b. In contrast to 1b the emulsion used contained only 2.04 g of silver (2-equivalent coupler). Samples of the finished layer were exposed and developed, both fresh and after cold storage under tropical conditions (for 7 days at  $35^{\circ}\text{C}/85\%$  relative humidity). The developer substance was again CD 1.

The following measurements were obtained:

|                        | relative sensitivity | density | fogging |
|------------------------|----------------------|---------|---------|
| fresh                  | 100                  | 1.70    | 0.09    |
| after tropical storage | 90                   | 1.62    | 0.11    |

Absorption maxima and secondary color densities

| Abs. max. | Absorption (%) |      |       |     |
|-----------|----------------|------|-------|-----|
|           | (nm)           | blue | green | red |
| CD 1      | 418            | 100  | 2     | 0   |
| CD 2      | 428            | 100  | 2     | 0   |
| CD 3      | 423            | 100  | 3     | 1   |
| T 60      | 422            | 100  | 4     | 0   |

c. Comparison test with the coupler:



according to the British Pat. No. 733,260.

This coupler had the tetradecyloxy group in the para position. Treatment as in 2a and 2b gave the following results:

|                  | relative sensitivity | density | fogging |
|------------------|----------------------|---------|---------|
| fresh            | 100                  | 1.79    | 0.63    |
| tropical storage | 110                  | 1.76    | 0.55    |

In contrast to coupler 18 used according to the invention, this coupler is remarkable for the high fogging levels of the fresh and stored materials.

Absorption maxima and secondary color densities

| 25   | Abs. Max. (nm) | Absorption (%) |       |     |
|------|----------------|----------------|-------|-----|
|      |                | blue           | green | red |
| CD 1 | 431            | 100            | 7     | 3   |
| CD 2 | 441            | 100            | 3     | 0   |
| CD 3 | 438            | 100            | 4     | 0   |
| T 60 | 436            | 100            | 8     | 2   |

It is clear from this Table that the dyes have unfavourable spectral properties.

What we claim is:

1. A color photographic material which comprises at least one silver halide emulsion layer containing a yellow coupler of the formula



in which

R<sub>1</sub> represents a linear or branched hydrocarbon chain having at least 10 carbon atoms;

X represents chlorine;

R<sub>2</sub> represents halogen, cyano, -R<sub>3</sub>, -OR<sub>3</sub>, -COOR<sub>3</sub>, -CONH<sub>2</sub>, -CONHR<sub>3</sub>, -CON(R<sub>3</sub>)<sub>2</sub>, -SO<sub>2</sub>R<sub>3</sub>, -SO<sub>2</sub>NH<sub>2</sub>, -SO<sub>2</sub>NHR<sub>3</sub>, -SO<sub>2</sub>N(R<sub>3</sub>)<sub>2</sub> or -SO<sub>2</sub>F, and if two or more groups R<sub>2</sub> are present, they can be the same or different;

R<sub>3</sub> represents alkyl having 1 to 4 carbon atoms or aryl, and if two groups R<sub>3</sub> occur in the same radical, they can be the same or different; and

n represents 1, 2 or 3.

2. A color photographic material as claimed in claim 1 wherein the yellow coupler has the formula



in which R<sub>1</sub>, R<sub>2</sub>, X and n have the meanings given in claim 1.

3. Color photographic material as claimed in claim 1 which has a plurality of emulsion layers, the yellow coupler being present in the blue-sensitive layer.

\* \* \* \* \*